

## UNITED STATES PATENT OFFICE.

WILHELM PUNGS, OF LUDWIGSHAFEN-ON-THE-RHINE, AND THEODOR HELTHALER, OF GRANSCHUTZ, GERMANY, ASSIGNORS TO I. G. FARBENINDUSTRIE AKTIENGESELLSCHAFT, OF FRANKFORT-ON-THE-MAIN, GERMANY, A CORPORATION OF GERMANY.

## BLEACHING MONTAN WAX.

No Drawing. Application filed November 26, 1927, Serial No. 236,004, and in Germany December 3, 1926.

We have found that crude or deresinified Montan wax can be bleached in a simple manner by exposing it, in a condition of solution or suspension, to the anodic action 5 of an electric current, in the presence of electrolytes and oxygen transmitters. Suitable oxygen transmitters comprise, for example, compounds of chromium, cerium, vanadium, manganese and the like. It is preferable to 10 operate in a solution or suspension, which does not offer any high resistance to the current, for example in 40 per cent sulfuric acid, or in phosphoric acid.

It is not essential, though generally advisable, to insert a porous diaphragm between 15 the anode and the cathode, to prevent a loss of current. The porous diaphragm may be replaced by a partition of solid, impermeable material, such as glass, which does 20 not extend quite to the bottom of the electrolyzing vessel. The strength of the current is preferably maintained at from about 300 to 500 amperes per square metre of the anode, and the tension at the electrodes, 25 generally at between 3 and 5 volts.

Lead, for example, is found to be a very suitable electrode material, in which event lead peroxid is formed at the anode.

It is important that the Montan wax be 30 in a very finely divided condition which may be furthered, for example, by energetically stirring the bath containing the crude Montan wax during the action of the current, and employing an elevated temperature, preferably about 100° C. In order to ensure 35 better distribution, if necessary, volatile organic solvents such as benzine, benzene, and its derivatives and the like, or organic acids such as acetic acid, may be added to the Montan wax.

Montan wax bleached according to the 40 present invention possesses practically the same properties as that obtained, for example, according to German Patent No. 409,420, or U. S. application for Patent 45 Ser. No. 218,853, filed September 10, 1927, and like that, may be separated into various products for example in accordance with the application for U. S. Patent Ser. No. 218, 854, filed September 10, 1927.

50 The following example will further illus-

trate the nature of the said invention which however is not limited thereto.

## Example.

55

A leaden vessel is charged with 40 per cent sulfuric acid containing from about 10 to 100 grams of chromium sulfate in solution per litre. The leaden vessel serves as the anode, and is connected to the positive 60 pole of a source of electric current. The cathode may consist of any convenient metal which resists the action of the electrolytes, and is preferably so constructed that it may be used as a stirrer. After the solution in 65 the vessel has been warmed to about 90° C., the crude Montan wax is energetically stirred in and the current is switched on. The tension is from about 3 to 5 volts, and the current intensity up to 500 amperes per 70 square metre of the anode. The temperature is slowly raised to above 100° C., and the current intensity is slightly lowered towards the end of the bleaching process.

When the Montan wax has been sufficiently decolorized, the current is switched 75 off and the stirrer stopped. The purified Montan wax then floats on the surface of the liquid, and can be run off while hot or taken off when cold.

## What we claim is:

80

1. The process of bleaching Montan wax which comprises exposing Montan wax finely divided in an electrolyte in the presence of an oxygen transmitter to the anodic action of an electric current.

2. The process of bleaching Montan wax which comprises exposing Montan wax finely divided in an electrolyte of low electric resistance, which state of division is furthered by the addition of a volatile organic solvent, to the anodic action of an electric current in the presence of an oxygen transmitter.

3. The process of bleaching Montan wax 95 which comprises exposing Montan wax finely divided in an electrolyte of low electric resistance to the anodic action of an electric current in the presence of an oxygen transmitter while stirring and heating the mixture to about 100° C.

4. The process of bleaching Montan wax

which comprises exposing Montan wax finely divided in sulfuric acid of 40 per cent strength to the anodic action of an electric current in the presence of an oxygen trans-  
5 ferrer while stirring and heating the mixture to about 100° C.

5. The process of bleaching Montan wax which comprises exposing Montan wax finely divided in an electrolyte of low electric  
10 resistance to the anodic action of an electric current of an intensity of between 300 to 500 amperes per each square metre of the anode and of a tension of about 3 to 5 volts, in the presence of an oxygen trans-  
ferrer.

6. The process of bleaching Montan wax 15 which comprises exposing Montan wax finely divided in sulfuric acid of 40 per cent strength heated to about 100° C. to the anodic action of an electric current of an intensity of between 300 to 500 amperes per 20 each square metre of the anode and of a tension of about 3 to 5 volts, in the presence of an oxygen trans-  
ferrer while stirring.

In testimony whereof we have hereunto set our hands.

WILHELM PUNGS.  
THEODOR HELLTHALER.